

## UNITED STATES PATENT OFFICE

2,371,631

## LUBRICANT

Bert H. Lincoln and Gordon D. Byrkit, Ponca City,  
Okla., assignors to Continental Oil Company,  
Ponca City, Okla., a corporation of Delaware

No Drawing. Application January 4, 1941,  
Serial No. 373,166

5 Claims. (Cl. 252—48)

This invention relates to improvements in lubricants. More specifically, this invention relates to improved materials which, when added to lubricants, greatly increase their resistance to oxidation and formation of corrosive products during use and often improves other characteristics as well. This is a continuation-in-part of our co-pending application, Serial No. 230,661, filed September 19, 1938.

Present-day mechanical devices require lubricating oils of high film strength and of high oiliness characteristics. It has been found that the present-day hydrocarbon lubricants of the very highest quality are deficient in these two very important characteristics. These two properties are of vital importance under conditions of thin film lubrication where the lubricant has been squeezed from between the friction surfaces because of high pressure, slow speeds, and other causes. It is readily seen that the viscosity or the body of the lubricant plays no part in this type of lubrication and that the remaining film of oil must have a very high film strength and be of high oiliness value to prevent rupture of the film of the lubricant, which would cause seizure. The oil film must tend to keep the coefficient of friction as low as possible.

Mechanical devices are being designed for higher pressure operation, and the film strength of the best quality straight hydrocarbon lubricant has been found to be too low. It will be obvious that an invention which provides a means of improving the film strength of these lubricants is of great importance to the art of lubricant manufacture and to the designer and fabricator of mechanical devices.

Substantially all machines operate in part or at times totally under conditions of boundary or thin film lubrication, under which conditions the oiliness or unctuousness of the lubricant is the first and primary requisite of efficient operation. Those skilled in the art of lubricant manufacture or machine manufacture will readily appreciate the value of an invention that will improve the oiliness of these otherwise high-quality lubricants.

In starting idle mechanical equipment which is lubricated from a sump by pumping or circulating the lubricant, there is always a short period of time in which the rubbing surfaces must operate under conditions of dry friction if ordinary hydrocarbon lubricants are used. With dry friction, the wear on friction surfaces is extreme; and during cold weather when the lubricant is sluggish or during periods when the lubricating system is not functioning properly for one reason or another, rubbing surfaces may not only suffer considerable wear but may be damaged to the point where they must be replaced. The product of our invention has a very important property

of reacting with the metal surfaces, penetrating or adsorbing on the metal surfaces, and leaving a film of lubricant with high oiliness character, which remains on the metal surface irrespective of the length of time the machine has been idle.

This high oiliness film gives very even and smooth operation, which may be easily discerned by the experienced operator or lubricating engineer.

10 When the hydrocarbon lubricants are diluted with unburned fuel or with other light hydrocarbons, the small degree of oiliness of the original hydrocarbon lubricant is greatly decreased. We have found that the addition of the products 15 of our invention to hydrocarbon lubricants more than compensates for the loss in oiliness and load-carrying ability from dilution.

It is well known that, in order to obtain lubricants which are preeminently satisfactory from 20 the standpoint of oxidation in use, it is necessary to refine the oil thoroughly and then to add an inhibitor of oxidation. The thorough refining may consist of more and heavier acid treatments or solvent treating so as to remove a considerable part of the oil and leave only the most stable portion. Such drastic refining is necessary in order to obtain stability with respect to sludge formation, but the oil is then subject to easy oxidation to form soluble acids and other 25 corrosive materials. It is practically impossible to refine an oil so as to avoid all of these difficulties. It is better to refine the oil thoroughly and then add small amounts of materials which either prevent the formation of these corrosive products or by some action render them inert.

Many of these additive materials are effective when added to poorly refined or even wholly unrefined lubricants. The addends may thus be substituted in whole or in part for the usual 30 refining processes.

In the prior art of applying these principles to the manufacture of lubricants, many diverse types of materials have been suggested to be added to obtain improvement in various characteristics, 45 but the esters of phosphorus acids with certain polyhydroxy organic compounds form a new type of material. We have found that the addition of these organic esters of the oxygen and sulfur acids of phosphorus improves film strength, oxidation resistance, noncorrosiveness, and other characteristics to an exceptional degree.

One object of our invention is to provide improved inhibitors of oxidation and corrosion for addition to lubricants.

55 Another object of our invention is to provide film strength improving addition agents suitable for use in lubricants and especially in crankcase lubricants.

Other and further objects of our invention will appear in the course of the following description.

Briefly our invention consists in the addition of esters of phosphorus acids and certain polyhydroxy organic compounds to hydrocarbon fuels and lubricants. By polyhydroxy organic compounds in the specification and appended claims, we include compounds containing two or more hydroxyl groups per molecule. According to our invention, the polyhydroxy organic compounds contain carbon, hydrogen, oxygen, and at least one other element. The fourth element may be chlorine or one of the other halogens, sulfur, or nitrogen. Esters of these substituted polyhydroxy organic compounds contain considerably more phosphorus than esters of monohydroxy organic compounds and are thus considerably more efficient. The negative element (halogen, sulfur, or nitrogen) in the organic radical apparently functions to make the phosphorus a more effective improver of film strength and/or inhibitor of oxidation. Some of the esters which are suitable for use according to our invention are chlororesorcinol phosphate, chloroethylene glycol phosphate, chlorocyclohexandiol phosphate, triethanolamine phosphite, thioglycol thiophosphate, and thioglycol phosphite.

Any of these compounds or other members of the classes represented or their derivatives within the limitations set forth above may be used within the scope of our invention. It will be noted that in addition to the elements C, H, O, and P our products contain halogen, sulfur, and/or other elements as well.

These materials form viscous liquids rather than crystalline products even when pure reactants are used. This is due to the heterogeneity in the number of reacting groups in the acid and polyhydroxy compound respectively. Reaction mixtures in which these compounds are being formed become more and more viscous as the reaction proceeds. We believe that the first esterification reaction produces high molecular weight linear condensation products of the type (taking chloroethylene glycol and phosphoric acid, for example, as the reactants):



Further reaction produces third dimensional condensation products:



Heating the reactants further produces branches again on the preformed chains until an extremely large and viscous macro-molecule results. We believe it is this unique type of structure of our products which lends such striking properties of film strength, viscosity index improvements, low cold test, and stability toward oxidation and formation of corrosive products during use when

blended with ordinary lubricants. It will be obvious to those skilled in the art that such a structure is impossible in the phosphorus esters of monohydric alcohols, phenols, and the like.

Compared with other esters of the acids of phosphorus and with other types of addends for lubricating oils, our materials are more stable to heat, pressure, and oxidation. When blended in lubricants, they produce oils which are less corrosive and less likely to form sludge and to stick rings in internal combustion engines.

It is to be understood that in practicing our invention oil-soluble esters of the type described are to be selected. Some of the examples described have only limited solubility in hydrocarbon oils. It is to be remembered, however, that, because of their great efficiency, extremely small amounts are often effective. Thus we may use as little as 0.001 per cent of some of these compounds, and it will be seen that a fairly insoluble material may dissolve to a sufficient extent to be satisfactory for our purpose. In general, more than 0.001 per cent of our addition agents are used; and we may add one, two, or even five per cent or more.

Furthermore, it is well known that different types of oils have different capabilities of dissolving a given material. For some purposes therefore, we prefer paraffinic, for other purposes asphatic, naphthenic or mixed base lubricants. Another method of obtaining a satisfactory mixture of addition agent with the hydrocarbon oil is the use of a mutual solvent to bring the addend into solution. Alternatively, peptizing agents may be added to maintain the ester in permanent suspension.

Many of the more difficultly soluble materials are rendered more soluble by the introduction of alkyl groups, particularly those containing four or more carbon atoms. The isoamyl, octyl, lauryl, and octadecyl radicals and radicals from paraffin wax greatly increase the solubility of organic compounds in oil. One or more of such groups may be introduced as required. For example, chlorohydroquinone phosphate is not very soluble in hydrocarbon lubricating oils but triamyl chlorohydroquinone phosphate is much more soluble.

The selection of a particular compound or compounds to be used as an addition agent to the hydrocarbon oil is to be made considering the use to which the blend is put. If a particular added phosphorus compound proves too volatile for its application, a higher boiling phosphorus compound should be used and the more volatile compound used for blending in a hydrocarbon oil intended for duty at lower temperature. In general, we prefer to use compounds having boiling points over 250 degrees F.

It is sometimes advantageous to combine more than one of these compounds in a blend to obtain particular properties. We accomplish this by mixing two or more of these compounds together and blending the mixture with the hydrocarbon oil or by blending one in the hydrocarbon oil, blending the second into this mixture, and so on until the composition is complete.

The esters of the type described usually improve both the film strength and oxidation characteristics of the hydrocarbon oil. For example, the sludging tendencies may be decreased by as little as 0.001 per cent of our phosphorus esters. The oxidation characteristics of lubricants are very important, and these are markedly improved by our compounds. The ability to reduce fric-

tion is another feature contributed to lubricants by our phosphorus esters.

It is usually desirable to include in one and the same blend based on a hydrocarbon oil, in addition to the addends here described, other addends for specific purposes. Thus we may add a pour point depressor such as a naphthalene-chlor wax condensation product and a viscosity index improver such as certain resins or polymerized hydrocarbons in addition to our phosphorus esters. Furthermore, various metallic compounds may be added to the blend without interfering with the action of our ingredients. Indeed, in some cases it is advantageous to combine with our phosphorus esters in a hydrocarbon oil blend such materials as calcium dichlorostearate, chromium oleate, tin octadecyl phthalate, aluminum stearate, and other metallic soaps.

Our addends are admirably adapted for use in lubricating oils of all types including those designed for use in automotive crankcases, Diesel oils, and any other oils of lubricating viscosity. By an oil of lubricating viscosity in the appended claims, we mean to include the so-called hydrocarbon or mineral oils, animal and vegetable oils, including castor oil, corn oil, soybean oil, lard oil, fish oils, and various synthetically treated oils including aluminum chloride treated oils, hydrogenated oils, voltolized oils, and all types of synthetic lubricants. Our addends are advantageously blended in gasoline and other fuels either directly or after being blended first in a lubricating oil and then added to the fuel. Soap-thickened mineral oils of all types ranging from those showing only a slight increase in viscosity over that of the mineral oil alone to the semi-solid and solid greases containing fifty per cent or more of soap are amenable to treatment according to our invention. In making these greases, the usual soaps such as sodium stearate, aluminum stearate, calcium soaps of beta fat, and the like may be used. Various other thickening ingredients for other purposes may be added. These include yarn, hair, graphite, glycerol, water, lampblack, mica, zinc dust, litharge, and the like.

The following examples of blends of our addition agent are given as illustrations and not as limitations:

*Example 1*

|                                         | Per cent |
|-----------------------------------------|----------|
| Mid-Continent paraffin base S. A. E. 30 | 99.0     |
| Chloro-ethylene glycol phosphate        | 1.0      |

*Example 2*

|                                      | Per cent |
|--------------------------------------|----------|
| Mid-Continent mixed base S. A. E. 30 | 98.4     |
| Aluminum naphthenate                 | 1.3      |
| Chlororesorcinol phosphate           | 0.3      |

*Example 3*

|                                                  | Per cent |
|--------------------------------------------------|----------|
| Paraffin base bright stock                       | 58.0     |
| Paraffin base neutral oil                        | 40.0     |
| Sulfurized methyl esters of corn oil fatty acids | 0.2      |
| Thiodiglycol phosphite                           | 0.3      |
| Calcium dichlorostearate                         | 1.0      |
| Diphenyl-chlorwax condensation product           | 0.5      |
|                                                  | 70       |

*Example 4*

|                                         | Per cent |
|-----------------------------------------|----------|
| Mid-Continent paraffin base S. A. E. 40 | 93.8     |
| Voltolized soybean oil                  | 5.0      |
| 5 Chlorodiphenylene oxide               | 1.0      |
| Triethanolamine phosphite               | 0.2      |

*Example 5*

In making a grease containing our addends, 10 we may use:

|                                            | Per cent |
|--------------------------------------------|----------|
| Oleic acid                                 | 8.1      |
| Lime                                       | 1.2      |
| Water                                      | 0.3      |
| 15 Dichlorostearic acid                    | 1.1      |
| Bright stock                               | 13.1     |
| Distillate (440 seconds at 100 degrees F.) | 76.0     |
| Chloro-ethyl cellulose phosphate           | 0.2      |

*Example 6*

In making a lubricating gasoline, we blend 0.5 per cent of the product of Example 1 with gasoline. The product has the composition:

|                                  | Per cent |
|----------------------------------|----------|
| Gasoline                         | 99.5     |
| Oil                              | 0.495    |
| Chloro-ethylene glycol phosphate | 0.005    |

It will be understood that certain features and 30 sub-combinations may be employed without reference to other species or combinations. This is contemplated by and is within the scope of our claims. It is further obvious that various changes may be made in details within the scope 35 of our claims without departing from the spirit of our invention. It is therefore to be understood that our invention is not to be limited to the details described.

Having thus described our invention, we claim:

1. A lubricant comprising a major proportion 40 of oil of lubricating viscosity and a minor proportion of an ester of an acid of phosphorus and a polyhydroxy organic compound which contains an element selected from the group consisting of halogens, sulfur, and nitrogen directly attached to a carbon atom of the polyhydroxy compound, said ester increasing the resistance of the lubricant to oxidation and to the formation of corrosive products during use.

2. A lubricant comprising an oil of lubricating 45 viscosity and from 0.001 to 5 per cent of an ester of an acid of phosphorus and a polyhydroxy organic compound which contains an element selected from the group consisting of halogens, sulfur, and nitrogen directly attached to a carbon atom of the polyhydroxy compound, said ester increasing the resistance of the lubricant to oxidation and to the formation of corrosive products during use.

3. A lubricant comprising a major proportion 55 of oil of lubricating viscosity and a minor proportion of chloro-resorcinol phosphate.

4. A lubricant comprising a major proportion 60 of oil of lubricating viscosity and a minor proportion of triethanolamine phosphite.

5. A lubricant comprising a major proportion 65 of oil of lubricating viscosity and a minor proportion of thiodiglycol phosphite.

BERT H. LINCOLN.  
GORDON D. BYRKIT.